

F. LANDGRAF,  
FLEXIBLE STAY BOLT FOR BOILERS.  
APPLICATION FILED FEB. 27, 1917.

1,256,911.

Patented Feb. 19, 1918.



WITNESSES  
Ed. V. Nollengaw  
G. F. Downing

INVENTOR  
F. Landgraf  
By Seymour & Bright  
Attorneys

# UNITED STATES PATENT OFFICE.

FREDERICK LANDGRAF, OF BRIDGEVILLE, PENNSYLVANIA, ASSIGNOR TO FLANNERY BOLT COMPANY, OF BRIDGEVILLE, PENNSYLVANIA.

## FLEXIBLE STAY-BOLT FOR BOILERS.

1,256,911.

Specification of Letters Patent. Patented Feb. 19, 1918.

Application filed February 27, 1917. Serial No. 151,251.

To all whom it may concern:

Be it known that I, FREDERICK LANDGRAF, a citizen of the United States, and a resident of Bridgeville, in the county of Allegheny and State of Pennsylvania, have invented 5 certain new and useful Improvements in Flexible Stay-Bolts for Boilers; and I do hereby declare the following to be a full, clear, and exact description of the invention, 10 such as will enable others skilled in the art to which it appertains to make and use the same.

This invention relates to the manufacture of flexible staybolts for boilers, and more 15 particularly to such as are made from tubular bars,—one object of my present invention being to provide a simple and efficient method of forming an integral spherical head at the outer end of a tubular iron body, 20 without contracting or interfering with the continuity of the bore which forms the tell-tale hole of the bolt from the inner end to the headed end of the bolt, and so that the outer end of said bore or tell-tale hole shall 25 terminate within and be closed by said integral head.

With this object in view, the invention 30 consists in certain novel features or steps in the method of making a flexible staybolt, as hereinafter set forth and pointed out in the claims.

In the accompanying drawings, Figure 1 35 is a view of a tubular bar from which the bolt is made; Fig. 2 is a view showing the first step in the method of forming the head; Fig. 3 is a view illustrating the next step with the integral spherical head formed on the bar; Fig. 4 is a view illustrating the bolt with the completely formed head with the 40 bore or tell-tale hole extending continuously from the inner end of the bolt to the headed outer end and terminating within the head, and Fig. 5 is a view illustrating the manner in which the outer end of the bore may be 45 closed prior to the forging of the head.

1 represents a tubular bar of iron, the bore 2 of which constitutes the tell-tale hole of the finished bolt.

In proceeding to form the spherical or 50 partly spherical head 3 on the outer end of the bolt, the end of the bar will be suitably heated and a mandrel 4 is inserted into the bore 2. The heating of the bar may be performed either before or after the insertion

of the mandrel. The mandrel may be 55 slightly tapering at its forward end, as indicated at 5, and if desired the mandrel may be coated with graphite to permit its ready removal after the head shall have been forged on the bar or bolt body. The mandrel 60 will be passed through the bore 2 until its forward end shall occupy a position therein which will be within the head subsequently forged. The tubular bar with the mandrel therein as above explained, will 65 next be subjected to the action of forging dies 6, whereby the metal at the outer end of the bar will be upset or forged to form the spherical or partly spherical head 3. The mandrel 4 may then be withdrawn as 70 shown in Fig. 4 and the bolt removed from the forging dies, and the headed bolt will have a tell-tale hole extending continuously from its inner end to the headed end and will terminate within and be permanently 75 closed by the integral head.

The bore may be closed at its outer end in any suitable manner before forging the head. Thus, a plug 7 may be secured in said outer end of the bore, as shown in Fig. 5, 80 and then the head may be forged as indicated by dotted lines, and during such forging operation, the plug will become welded in the head.

Having fully described my invention what 85 I claim as new and desire to secure by Letters-Patent, is:—

1. The herein described method of making a staybolt, consisting in inserting a mandrel partially through a tubular bar, forging a 90 head on said tubular bar and then withdrawing the mandrel, leaving the bore continuous from the inner end of the bolt and extending into the headed end and closed at the outer end of the bolt within the forged 95 head thereon.

2. The herein described method of making a staybolt, consisting in inserting a mandrel partially through a tubular bar, forging a head on said bar over and about the 100 forward end of the mandrel, and then withdrawing the mandrel, leaving the bore of the bolt continuous from the inner end of the bolt to a point within the forged head at the outer end of the bolt.

3. The herein described method of making a staybolt consisting in inserting a mandrel partially through a tubular bar closed 105

at one end, then forging a head on the closed end of said tubular bar and then withdrawing the mandrel leaving the bore continuous from the inner end of the bolt and extending into the headed end, and closed at the outer end of the bolt in the forged head thereon.

In testimony whereof, I have signed this specification in the presence of two subscribing witnesses.

FREDERICK LANDGRAF.

Witnesses:

H. M. SCHADEL,  
V. E. SKELLEY.

Copies of this patent may be obtained for five cents each, by addressing the "Commissioner of Patents, Washington, D. C."